

[54] **FREE MACHINING AUSTENITIC STAINLESS STEEL ALLOY**

[75] Inventors: **Kermit J. Goda, Jr., Leesport; Grant M. Aulenbach, Mohnton, both of Pa.**

[73] Assignee: **Carpenter Technology Corporation, Reading, Pa.**

[22] Filed: **Jan. 24, 1972**

[21] Appl. No.: **220,108**

**Related U.S. Application Data**

[63] Continuation-in-part of Ser. No. 855,416, Sept. 4, 1969, Pat. No. 3,645,722.

[52] **U.S. Cl.** 75/124, 75/125, 75/128 P, 75/128 R

[51] **Int. Cl.** C22c 39/20

[58] **Field of Search** 75/128 P, 124

[56] **References Cited**

**UNITED STATES PATENTS**

R23,685 7/1953 Clarke ..... 75/128 P  
3,152,934 10/1964 Lula ..... 75/124

|           |         |                  |          |
|-----------|---------|------------------|----------|
| R27,226   | 1/1970  | Moskowitz .....  | 75/128 P |
| 2,661,279 | 12/1953 | Wilcox .....     | 75/128 P |
| 3,362,813 | 1/1968  | Ziolkowski ..... | 75/124   |
| 1,961,777 | 6/1934  | Palmer .....     | 75/128 P |
| 2,697,035 | 12/1954 | Clarke .....     | 75/128 P |
| 3,151,978 | 10/1964 | Perry .....      | 75/124   |
| 3,340,046 | 9/1967  | Dulis .....      | 75/128 P |
| 3,408,178 | 10/1968 | Myers .....      | 75/124   |

*Primary Examiner*—Hyland Bizot  
*Attorney, Agent, or Firm*—Edgar N. Jay

[57] **ABSTRACT**

Austenitic stainless steel alloy containing about 10 percent to 26 percent chromium, 4 to 46 percent nickel, 0.4 to 15 percent manganese, 0.015 to 0.75 percent sulfur and/or selenium, 0.5 to 10 percent copper, 0.25 to 2 percent aluminum, 0.001 to 0.1 percent tellurium, and the balance being iron, optional elements and incidental impurities. Austenitic compositions are provided having improved free-machining properties or an improved combination of free-machining and corrosion-resistance properties in selected media.

**12 Claims, No Drawings**

## FREE MACHINING AUSTENITIC STAINLESS STEEL ALLOY

This application is a continuation-in-part of our co-pending application filed Sept. 4, 1969, Ser. No. 855,416 and now U.S. Pat. No. 3,645,722, granted Feb. 29, 1972.

This invention relates to stainless steel alloys and, more particularly, to austenitic stainless steel alloys having improved free machinability or improved combined properties of free machinability and corrosion resistance in selected media.

Austenitic stainless steel alloys may contain from about 10 to 26 percent chromium and 4 to 46 percent nickel. Because of their mechanical and chemical properties, such alloys are highly desired for a wide variety of uses, but, because of the difficulty encountered in machining such alloys, it has hitherto been the practice to modify standard grades by means of free-machining additives for use where the accompanying reduction in corrosion resistance could be tolerated. For example, A.I.S.I. type 303 and type 303(Se) are illustrative of grades which contain respectively substantial amounts of sulfur and selenium, that is more than about 0.15 percent and usually 0.3 percent or more, for improved machinability.

A number of other elements have also been used in combination with or in place of the elements sulfur and selenium, but the results left much to be desired, usually because the increase in the cost of the alloy and/or the detrimental effect on other properties such as corrosion resistance were not sufficiently offset by the gain in free-machining properties. Our present invention stems from our discovery that when a relatively small amount of tellurium is present together with the elements manganese, copper and aluminum, they work together with sulfur or selenium or both of them to impart a unique degree of free machinability to austenitic chromium-nickel stainless steel alloys without reducing the corrosion resistance to the extent expected from previous experience with the sulfur or selenium additions required to attain a like degree of machinability.

It is therefore a principal object of the present invention to provide an austenitic stainless steel characterized by an enhanced degree of free machinability compared to currently available corresponding grades of austenitic free-machining stainless steel and having at least about as good corrosion resistance.

By providing an austenitic chromium-nickel stainless steel alloy containing the elements indicated in the following broad range, much of the foregoing objects are achieved while the preferred range ensures attainment of the foregoing as well as additional objects, both ranges being given in approximate weight percent:

|                          | Broad Range | Preferred Range |
|--------------------------|-------------|-----------------|
| Carbon                   | up to 0.25  | up to 0.2       |
| Chromium                 | 10-26       | 10-20           |
| Nickel                   | 4-46        | 4-35            |
| Manganese                | 0.4-15      | 0.4-2           |
| (Sulfur and/or Selenium) | 0.015-0.75  | 0.02-0.35       |
| Copper                   | 0.5-10      | 0.75-4          |
| Aluminum                 | 0.25-2      | 0.5-1.25        |
| Tellurium                | 0.001-0.1   | 0.01-0.06       |

In addition, there can be included varying amounts of other elements, as for example: up to about 3 percent silicon but preferably no more than 1 percent, up to about 0.5 percent preferably no more than 0.035 percent phosphorus, up to about 3.5 percent molybdenum, or tungsten can replace all or part of the molybdenum in the ratio of about 2 to 1, up to about 0.01 percent boron, columbium up to about 10 times the percent carbon plus nitrogen but no more than about 2 percent, titanium in an amount up to about equal to six times the percent carbon plus nitrogen but no more than about 1.2 percent, and up to about 0.35 percent nitrogen. Except for incidental impurities, the balance of the alloy is iron.

15 The elements sulfur and/or selenium together with controlled amounts of manganese, copper, aluminum and tellurium work together in our composition to provide an unexpected degree of free machinability and corrosion resistance. While sulfur in amounts ranging from about 0.015 to 0.75 percent can be present, above about 0.5 percent increasing difficulty may be encountered in both hot and cold working the composition. Therefore, when necessary to minimize working difficulties, we limit sulfur to no more than about 0.4 percent and preferably to no more than about 0.35 percent. Selenium on a one-for-one basis can be substituted for all or part of the sulfur in our composition as is indicated in the foregoing tabulation where the ranges stated are to be read as the broad and preferred amounts of the combined content of both sulfur and selenium. The elements sulfur and selenium, individually or together, are not equivalent to and cannot be substituted for the element tellurium in our composition.

35 For its effect in contributing to free machinability, manganese preferably in an amount from about 0.4 to 2 percent is included in our composition, while best results can be obtained with about 1.4 to 1.6 percent. As is well known, manganese can be used in addition to or in place of part of the nickel content in establishing the austenitic balance in austenitic stainless steel alloys, and up to about 15 percent manganese can be used for that purpose in our alloy. Having in mind that free-machining stainless steel alloys are not intended for use where they would be exposed to very corrosive media, the best combination of corrosion resistance and free machinability is obtained with about 0.4 percent to about 0.7 percent manganese or, better yet, no more than about 0.6 percent. It is also to be noted that in order to improve the corrosion resistance of our composition when more than 0.7 percent manganese is present, parts formed therefrom can be passivated as by using 50 percent by weight nitric acid or other suitable passivating media. The manganese functions to increase the solubility of the sulfides (or selenides when the latter are present). The passivation treatment serves to remove the manganese sulfides (or selenides) from the surface of the treated part. Of course, if the passivated surface from which the manganese sulfides have been removed wears away in use, then the underlying material becomes exposed and is subject to attack.

60 Copper is present in solid solution in our composition and primarily appears to enhance the corrosion resistance of our alloy. The effect of copper on free machinability seems to result from lowering the work hardening rate. For this purpose we preferably use about 0.75 to 4 percent copper. Below about 0.5 percent, there is

not enough copper present to provide a significant effect while above about 10 percent increasingly severe segregation problems appear which cause hot shortness. The most beneficial effect of copper is its effect on improving the corrosion resistance of our alloy.

Aluminum contributes to the formation of smaller and thereby better dispersed sulfides, but only in the presence of an effective amount of tellurium. Because aluminum is a powerful ferrite former, its use must be carefully controlled in compositions like the present which are to be entirely or primarily austenitic. Broadly, from about 0.25 to 2 percent aluminum can be present in our composition. Larger amounts of aluminum make it increasingly difficult to preserve the austenitic balance of our composition. We prefer to use aluminum in an amount ranging from about 0.50 to 1.25 percent.

In the absence of at least a small but effective amount of tellurium, the outstanding free machinability of our composition cannot be attained. We preferably use about 0.01 to 0.06 percent tellurium although as little as 0.005 percent or even 0.001 percent can have an effect and as much as 0.1 percent tellurium can be used to some advantage. In spite of the fact that tellurium in the presence of sulfur but without the necessary amounts of manganese, aluminum and copper does not improve the free machinability of austenitic stainless steel and appears to detract from it, we have found that with the aluminum, manganese and copper present in our composition together with tellurium, there is an unexpected synergistic effect upon the free machinability of our composition as measured by the drill test.

We do not have a complete explanation for or completely understand the phenomenon, but based on our observations, it appears that the tellurium forms tellurium-rich compounds which we thus far have identified as tellurides that are attached to the sulfides. The more tellurium present, the more the sulfides are surrounded by the tellurium-rich compounds.

By the addition of the elements manganese, aluminum, copper and tellurium in accordance with our invention, the sulfur content of a given alloy can be reduced so as to obtain better corrosion resistance with little or no loss in free machinability or even in some

instances with some improvement in machinability. On the other hand, when the previously acceptable sulfur level is maintained, the addition of the elements manganese, aluminum, copper and tellurium, all within the stated ranges, makes possible significantly improved free machinability.

The examples having the analyses in approximate weight percent as shown in Table I serve to illustrate our invention.

10 Ingots were cast of each of the foregoing examples, hot worked and shaped to form test pieces which were annealed before testing. Our composition is wholly or predominantly austenitic both at room temperature and at the usual hot working temperature range for such alloys, that is from a furnace temperature of about 2,100° F. Preferably, ingots are first subjected to some light hot working to break up the as-cast structure. Then after surface preparation, e.g., grinding to remove surface checks, hot working is completed in the usual way from a furnace temperature of about 2,100° F. In the case of more difficult to work ingots, somewhat better results can be attained by sadding at a higher temperature, up to about 2,300° F.

20 Examples 1-6 were annealed at about 1,950° F for one hour followed by cooling in air. The hardness of the examples in their annealed condition was measured on the Rockwell B Scale, and the results are recorded at the bottom of Table I.

25 The machinability of the specimens of each of the examples was determined as the average depth of penetration in thousandths of an inch into the specimens under carefully controlled conditions. While there is no generally accepted standard for measuring machinability, the free machining values were obtained by measuring the depth of penetration into the specimens by a quarter-inch drill in a time interval of 15 seconds with the drill rotating at or very close to 670 r.p.m. under constant torque. Before the start of each drilling operation, the drill mounted in a conventional drill press was 30 brought against the surface of the specimen where it was maintained by a constant weight of 100 pounds. The results of the tests are recorded at the bottom of Table I as "Drill Test," and each is an average of two sets of seven tests.

TABLE I

|              | EXAMPLE NO. |        |        |       |        |        |
|--------------|-------------|--------|--------|-------|--------|--------|
|              | 1           | 2      | 3      | 4     | 5      | 6      |
| C            | .120        | .091*  | .120*  | .131  | .095*  | .095*  |
| Mn           | 1.72        | 1.63   | 1.68   | 1.68  | 1.67   | 1.68   |
| Si           | .45         | .51*   | .45*   | .39   | .44*   | .44*   |
| P            | .005        | .012   | .005*  | .012  | .012   | .012*  |
| S            | .31         | .27    | .31    | .27   | .27    | .24    |
| Cr           | 17.26       | 16.63* | 17.26* | 16.82 | 17.14* | 17.14* |
| Ni           | 10.00       | 10.06  | 10.00* | 10.08 | 9.81*  | 9.81*  |
| Mo           | .01         | .01*   | .01*   | .01   | .01*   | .01*   |
| Al           | .84         | .50    | .67    | .41   | .92    | .92    |
| Cu           | .85         | 1.47   | 1.68   | .79   | .74    | 1.49   |
| Te           | .001        | .004   | .016   | .04   | .04    | .04    |
| N            | .037        | .046   | .037*  | .032  | .042*  | .042   |
| Rockwell B   | 79.5        | 80     | 78     | 81    | 86     | 84.5   |
| Drill Test** | 547         | 455    | 474    | 482   | 575    | 568    |

\*For economy, the heats were split to permit variation in the elements Mn, S, Al, Cu and Te. The asterisk indicates analyses of elements obtained by measurement from other portions of the same heat to avoid unnecessary analysis.

\*\*In thousandths of an inch.

For comparison, the following alloys were prepared, formed into specimens and tested as was described in connection with Examples 1-6.

|           |      |
|-----------|------|
| Boron     |      |
| Columbium | 0.01 |
| Titanium  | 2    |
| Nitrogen  | 1.2  |
| do.       | 0.35 |

TABLE II

|                | A      | B      | C      | D     |
|----------------|--------|--------|--------|-------|
| C              | .101   | .107   | .108*  | .115  |
| Mn             | .07    | 1.47   | 1.76   | 1.69  |
| Si             | .24    | .31    | .43*   | .38   |
| P              | .007   | .007   | .006*  | .006  |
| S              | .37    | .42    | .32    | .31   |
| Cr             | 16.95  | 17.02  | 17.19* | 17.09 |
| Ni             | 9.76   | 9.79   | 9.79*  | 9.79  |
| Mo             | .02    | .02    | .02*   | .01   |
| Al             | <.01   | <.01   | .36    | .92   |
| Cu             | .05    | .06    | .76    | 1.54  |
| Te             | <.0002 | <.0002 | <.0002 | <.001 |
| N <sub>2</sub> | .043   | .045   | .036   | .038  |
| Rockwell B     | 88.5   | 88     | 85     | 81.5  |
| Drill Test**   | 338    | 429    | 423    | 443   |

\*For economy, the heats were split to permit variation in the elements Mn, S, Al, Cu and Te. The asterisk indicates analyses of elements obtained by measurement from other portions of the same heat to avoid unnecessary analysis.

\*\*In thousandths of an inch.

Alloy A shows the effect of sulfur in such a chromium-nickel austenitic stainless steel with low manganese and without an addition of aluminum, copper and tellurium. With a hardness of R<sub>b</sub>88.5 in the annealed condition, the average drill test penetration of Alloy A was found to be .338 inch. Alloy B primarily demonstrates the effect of adding manganese in increasing the average drill test penetration to .429 inch, but the increase in sulfur from .37 to 42 percent also contributed its relatively small effect. Alloys C and D demonstrate that the addition of the elements aluminum and copper does not provide a synergistic effect with manganese and could result in a reduction in free machinability if tellurium is not added in accordance with our invention. On the other hand, Example 1, which has virtually the same analysis as Alloy D except for the small addition of tellurium, gave an average drill test penetration of .547 inch. See also Example 2 which, with only .27 percent sulfur and .004 percent tellurium, gave an average drill test penetration of .455 inch. The as-tested hardness of the specimens of Examples 1 and 2, and Alloy D ranged from R<sub>b</sub>79.5 to R<sub>b</sub>81.5 and thus were not considered to differ significantly.

The terms and expressions which have been employed are used as terms of description and not of limitation, and there is no intention in the use of such terms and expressions of excluding any equivalents of the features shown and described or portions thereof, but it is recognized that various modifications are possible within the scope of the invention claimed.

We claim:

1. An austenitic stainless steel alloy having good free machinability in its annealed condition consisting essentially in weight percent of about:

|                      |             |
|----------------------|-------------|
| Chromium             | 10-26       |
| Nickel               | 4-46        |
| Sulfur plus Selenium | 0.015-0.75  |
| Copper               | 0.5-10      |
| Aluminum             | 0.25-2      |
| Tellurium            | 0.001-0.1   |
| Manganese            | 0.4-15      |
| Carbon               | up to about |
| Silicon              | do.         |
| Phosphorus           | do.         |
| Molybdenum           | do.         |

in which an equivalent amount of up to about 7 percent tungsten in the ratio of about 2/1 can replace all or part of the molybdenum, and the balance essentially iron.

2. The austenitic stainless steel alloy as set forth in claim 1 containing about 0.02-0.5 percent sulfur plus selenium, about 0.4-2 percent manganese, about 0.75-4 percent copper, about 0.5-1.25 percent aluminum, and about 0.005-0.06 percent tellurium.

3. The austenitic stainless steel alloy as set forth in claim 2 containing about 1.4-1.6 percent manganese.

4. The austenitic stainless steel alloy as set forth in claim 1 containing about 0.4-2 percent manganese.

5. The austenitic stainless steel alloy as set forth in claim 4 containing about 0.5-4 percent copper.

6. The austenitic stainless steel alloy as set forth in claim 5 containing about 10-20 percent chromium, and about 4-35 percent nickel.

7. The austenitic stainless steel alloy as set forth in claim 6 containing no more than about 1 percent silicon, and no more than about 0.035 percent phosphorus.

8. The austenitic stainless steel alloy as set forth in claim 2 containing about

|            |             | Weight Percent |
|------------|-------------|----------------|
| Chromium   |             | 10-20          |
| Nickel     |             | 4-35           |
| Carbon     | up to about | 0.2            |
| Silicon    | do.         | 1              |
| Phosphorus | do.         | 0.035          |
| Columbium  | do.         | 10x(% C+N)     |
| Titanium   | do.         | 6x(% C+N)      |

9. The austenitic stainless steel alloy as set forth in claim 8 containing about 1.4-1.6 percent manganese.

10. The austenitic stainless steel alloy as set forth in claim 8 containing about 0.02-0.35 percent sulfur plus selenium.

11. The austenitic stainless steel alloy as set forth in claim 10 containing about 0.01-0.06 percent tellurium.

12. The austenitic stainless steel alloy as set forth in claim 11 containing about 0.4-0.7 percent manganese.

\* \* \* \* \*